

Feb. 9, 1937.

W. G. MARTIN

2,070,368

## METHOD FOR ENAMELING TANKS

Filed June 8, 1935

2 Sheets-Sheet 1



INVENTOR.

INVENTOR  
*Wesley G. Martin*

BY Elwin C. Andrews

ATTORNEY.

Feb. 9, 1937.

W. G. MARTIN

2,070,368

METHOD FOR ENAMELING TANKS

Filed June 8, 1935

2 Sheets-Sheet 2

FIG. 2.



FIG. 3.



INVENTOR.

Wesley G. Martin

BY *Clavin C. Andrus*

ATTORNEY.

## UNITED STATES PATENT OFFICE

2,070,368

## METHOD FOR ENAMELING TANKS

Wesley G. Martin, Milwaukee, Wis., assignor to  
 A. O. Smith Corporation, Milwaukee, Wis., a  
 corporation of New York

Application June 8, 1935, Serial No. 25,694

8 Claims. (Cl. 91—73)

This invention relates to the application of vitreous enamel linings to the interiors of tanks such as are used for the storage of beer, or milk, or other liquids which would be contaminated by contact with metal.

An object of the invention is to provide an improved method for the application of vitreous enamel coatings to the interiors of tanks.

A further object of the invention is to provide suitable apparatus for use in connection with the method.

Other objects of the invention will be clear from the following detailed description and the accompanying drawings, in which:

Figure 1 is a side elevation of a tank within a furnace during the fusing of the enamel;

Fig. 2 is a side elevation, partly in section, of the apparatus used in carrying out the method of this invention, and constitutes an enlarged view of the left hand portion of Figure 1;

Fig. 3 is a top plan view of the apparatus;

Fig. 4 is an enlarged sectional view taken on line 4—4 of Fig. 3; and

Fig. 5 is a sectional view taken on line 5—5 of Fig. 4.

The application of a vitreous enamel lining to the interior of a tank presents a number of serious difficulties. A tank some eleven feet in diameter and thirty feet long has an internal surface in excess of one thousand square feet, and this surface should be completely covered with a faultless coating of enamel in one firing. Defects in the enamel coating which may be small in area may nevertheless require the application of another coat of enamel to the entire inner surface of the tank, and another firing in order to produce a tank which will be satisfactory for the purpose for which it is desired. Due to the large size of the tanks which may be involved, a large expense is involved in an additional firing to cure any defects which may exist in a previously applied coat of enamel. For this reason it is desirable to have methods available which will reduce to a minimum the possibility of defects in an enamel lining of a tank.

One of the objects of my invention is to provide a method for enameling tanks which will enable a satisfactory lining of enamel to be applied in a single coat. A single coat lining is preferable to a multiple coat lining on the ground of greater cheapness, and for some applications has other points of superiority as well, such as lesser thickness and greater resistance to injury by mechanical shock. In some cases a multiple coat lining may be preferred for particular rea-

sons. The methods of this invention are of no less value for the production of such multiple coat linings, for it is axiomatic in the enameling industry that the ground coat should be as faultless as it can be made. While blisters and copperheads or other defects in the ground coat may sometimes be covered up by the subsequently applied coats of enamel, this by no means invariably occurs. Furthermore, a defective ground coat may reboil when the other coats are applied and in this way give rise to serious difficulty in the production of a satisfactory enamel lining.

In my co-pending application for patent, Serial No. 730,063, filed June 11, 1934, and since issued as U. S. Letters Patent No. 2,004,632, I have disclosed that difficulties which are frequently encountered when an enamel is burned in air may be avoided if the enamel is fused to its metal base in an atmosphere substantially devoid of free oxygen. Steels which give rise to such defects as copperheads or blisters, or which cause reboiling when the enamel is fused in air, can be satisfactorily enameled if the enamel is burned in a suitable atmosphere substantially devoid of free oxygen as disclosed in my co-pending application. Carbon dioxide is an example of a suitable atmosphere which is disclosed in that application.

The present invention is concerned specifically with methods and apparatus for the convenient and rapid expulsion of free oxygen from within the tank which is being fired. In carrying out the method of this invention, it is preferred to first heat the tank while it is filled with air in order to produce a film of oxide on the inner surface of the metal tank, and to then replace the air by a different gas before the temperature has risen sufficiently to fuse the enamel.

According to this invention the air initially within the tank is driven out and replaced by another gas by introducing this gas into the heated tank in solid form. This method of filling the tank with gas possesses a number of important advantages. The solidified gas is itself of small volume but expands enormously when it is vaporized in the tank. Many of the tanks which are enameled on the inside are of very considerable dimensions and have a volume of several thousand cubic feet. It is desired to drive out the air and replace it with a different gas in the course of a few minutes. If gas were pumped into the tank to drive out the air it would be necessary to either supply a large pipe leading from the tank to the outside of the furnace in which it is heated, or, in case a small pipe is used, to employ a very

high gas velocity. Neither of these expedients is desirable. By using gas in the solid form these difficulties are avoided. The atmosphere desired in the tank is introduced in condensed form and 5 expands in volume after it is within the tank.

Carbon dioxide is an example of a gaseous atmosphere which is suitable for the burning of enamels. For use in connection with this invention, carbon dioxide has the additional advantage 10 that it can be readily obtained in the solid form, the well known "dry ice" of commerce being solidified carbon dioxide gas.

A further advantage is that small chips of solid 15 carbon dioxide blown into the tank tend to settle to the bottom because of their weight. Since the tank is hot when the solid carbon dioxide is introduced, it is rapidly converted into gas. This will occur at or near the bottom of the tank. Since 20 carbon dioxide is a much heavier gas than air it will lie beneath the air initially within the tank and rise beneath it. It is, of course, not to be expected that there will be no mixing of carbon dioxide gas with air but it will be readily appreciated that there will be much less admixture and 25 much more effective utilization of the carbon dioxide if it is introduced at the bottom of the tank. The openings provided for the exit of air should be located at the top of the tank.

In enameling a tank according to my improved 30 method, the tank is first made and prepared for enameling. In case the tank is fabricated from sheet steel by electric arc welding with certain kinds of electrodes, it is desirable that the welded tank be treated according to the methods disclosed in my co-pending application, Serial No. 35 25,695, filed on even date herewith, in order that no difficulty may be experienced in getting the enamel to adhere to the electric arc welds. After the tank has been thus treated, the inside is sandblasted, imperfections uncovered in the steel 40 plates are ground out, and the ground patches are preferably sandblasted again. The sand is cleaned from the tank and a coat of enameling material is applied to its inner surface by any 45 suitable method, as by spraying. Any suitable enameling material can be used. The coating of enameling material is then dried. This may be conveniently done by passing a current of filtered air through the tank and heating the outside with 50 a large gas flame.

Suitable covers are provided for the openings in the tank. These should desirably be made as tight as possible. One of the openings is provided with an inlet pipe of sufficient length to reach 55 well beyond the furnace when the tank is placed within the furnace for firing. The opening to which the inlet pipe is connected should preferably be near the bottom of the tank. One of the openings at the top of the tank is provided with a 60 valve which is originally open to permit the escape of air but which can be closed by a wire leading outside the furnace.

Thus equipped, the tank is placed on a car and introduced into a furnace for fusing the enamel. 65 The inlet pipe extends beyond the furnace and is connected to suitable apparatus for introducing solid carbon dioxide chips into the tank.

Referring to Fig. 1, the tank 1 is shown supported on car 2 within the furnace 3 in which 70 the enamel is fused. The furnace may be heated by any suitable means as by electricity or the combustion of fuels. An opening 4 near the bottom of the tank is covered by a manhole cover 5 to which the inlet pipe 6 is fastened. Another 75 opening 7 near the top of the tank is provided

with a valve 8 which can be closed by wire 9. A small tube 10 is connected to the inlet pipe 6 near the tank. At its outer end the pipe 10 is connected to a water manometer 11 for measuring the pressure differential between the gas within 5 the tank and the outside atmosphere.

The outer end of the inlet pipe 6 is secured to a connector 12 which has a branch inlet 13. The branch inlet 13 is secured to a hose 14 for supplying air or other gas under pressure, and the connector 12 is secured to a tube 15 which leads to the apparatus 16 for introducing solid carbon dioxide chips into the tank. Valves 17 and 18 are provided to enable the inlet pipe 6 to communicate with either of the connecting pipes 14 and 15, or 15 to be shut off from both.

The apparatus 16 for converting blocks of solid carbon dioxide into chips or shavings and injecting them into the tank comprises a rectangular box 19 supported on a suitable framework 20. A 20 flanged opening 21 is provided at the top of the box to permit the introduction of blocks of solid carbon dioxide into the machine. A cover 22 is provided to close the box after it is filled with carbon dioxide blocks. The cover bears on gasket 25 23 and is held in place by clamps 24, thus assuring a tight joint.

A plunger 25 fitting within the box 19 is carried on a piston rod 26. A piston 27 secured to the piston rod 26 travels in the air cylinder 28. 30 By means of the valve 29 and ports 30 and 31, air from a compressed air line 32 can be admitted to either end of the air cylinder 28. The piston rod 26 travels through stuffing boxes 33 and 34 which prevent leakage from the air cylinder 28 35 and the box 19 respectively.

The end of the box 19 opposite the air cylinder is secured to an approximately cylindrical casing 35. A toothed cylinder 36 is supported within this casing by shaft 37 running in bearings 38. The toothed cylinder is driven in the direction indicated in Figs. 2 and 4 by an electric motor 39 supported on brackets 40.

The lower side of the cylindrical casing 35 is connected to the fan-shaped outlet 41 which in 45 turn connects with the tube 15. At the wide end of the outlet 41 is placed a block 42 extending the full width of the outlet. This block has a longitudinal chamber 43 with which forwardly directed openings 44 communicate.

The rotating cylinder 36 has teeth provided on its outer surface for shaving chips of carbon dioxide from carbon dioxide blocks 45 placed in the box 19 and forced against the cylinder by the plunger 25. Gas under pressure is admitted to the chamber 43 in the block 42 and upon escaping through the openings 44 in block 42 carries the carbon dioxide chips through the outlet 41 to pipe 15, and from there through the valve 18 and pipe 6 to the tank 1. The gas used 60 to blow the chips into the tank may be provided in any suitable way as by a small gas producer operated under pressure to produce an atmosphere composed essentially of carbon dioxide and nitrogen, or by a compressor forcing flue gas into 65 the block 42; or, as indicated in the drawings, by a battery of liquid carbon dioxide cylinders 46. These cylinders are connected through valves 47 and pipes 48 to a header 49 which communicates with the chamber 43. An orifice 70 or Venturi meter (not shown in the drawings) may desirably be inserted in the line leading from the header 49 to the chamber 43 to indicate the rate at which carbon dioxide is being drawn from the cylinders. When carbon dioxide 75

cylinders are used it is desirable that several be connected together so that they can be used in turn. An excessive drain from any one cylinder results in a lowering of its temperature and 5 may cause its contents to freeze.

A gas burner 50 supplied with gas by tube 51 may desirably be placed below the box 19 to keep the carbon dioxide blocks 45 from freezing to the bottom of the box.

10 Tie rods 52 connected to the framework of the apparatus lead to an eye 53 by means of which the whole equipment may be readily lifted with a crane and placed in any desired position.

In using the method and apparatus of this 15 invention, the tank to be lined with enameling material is provided with coverings for the openings and with an inlet pipe 6 as previously described, and is placed upon the car 2. The car is then run into the heated furnace 3 and the 20 tank begins to heat up. The apparatus for injecting solid carbon dioxide into the tank is connected to the pipe 6. As the tank heats up the air which it initially contained expands and escapes through the opening 7 and valve 8.

25 After the tank has been sufficiently heated to cause the formation of a thin film of oxide on the inner wall of the tank, the motor 39 is started and air pressure is admitted to the left hand end of the air cylinder 28 to force blocks of 30 carbon dioxide previously placed in the box 19 against the rotating toothed wheel 36. One or more of the valves 41 is opened to provide a current of gas from carbon dioxide cylinders 46 to blow the chips shaved from the carbon dioxide 35 blocks by the rotating cylinder into the tank. The carbon dioxide chips are vaporized by the heat of the tank, and the gas which is formed forces the air out through the valve 8. The rate of admission of carbon dioxide to the tank 40 is controlled by the manipulation of valve 29 allowing air to enter the air cylinder 28 and is so regulated that the gas pressure within the tank does not exceed a value which the tank can safely withstand while in a heated condition.

45 After a sufficient amount of carbon dioxide to drive out the air has been admitted to the tank, the valve 8 is closed by pulling on the wire 9. The closure of the valve will greatly diminish 50 the rate at which gas can escape from the tank but there will ordinarily be sufficient leakage to require the continued gradual admission of carbon dioxide in order to maintain the pressure within the tank somewhat above the atmospheric 55 pressure. The gradual admission of carbon dioxide may be effected by reducing the rate at which solid carbon dioxide chips are blown into the tank, or the valve 18 may be closed and clean flue gas under pressure admitted through 60 the valve 17 which is so regulated as to maintain a suitable pressure within the tank. Flue gas consists predominantly of carbon dioxide and nitrogen and when cleaned of solid particles which might deposit upon and injure the enamel, is a suitable atmosphere for the burning of 65 enamels; but it will not, of course, as rapidly replace the air within the tank as will carbon dioxide which can be introduced in solid form.

70 After the tank has been heated to a sufficient temperature to fuse the enamel, it is no longer indispensable, although it is preferable, to maintain within the tank an atmosphere which is substantially devoid of free oxygen. Hence, when this stage has been reached air can be admitted through the valve 17 to maintain a 75

slight pressure within the tank. It is desirable that an excess pressure be maintained within the tank while it is in a heated condition because this helps to maintain its shape.

With the particular furnace which has been 5 used, some forty to forty-five minutes was taken for firing a tank about eleven feet in diameter and thirty feet long with walls  $\frac{1}{4}$ " in thickness. About five minutes after the tank was run into the furnace the admission of carbon dioxide was 10 begun and was continued at a sufficient rate to maintain a few inches of water pressure within the tank. The valve 8 was closed about twenty minutes after the tank entered the furnace. This reduced the rate of escape of gas from the 15 tank. Carbon dioxide was admitted slowly to make good the loss of gas by leakage and to maintain within the tank about the same pressure as before. About twenty-five minutes after the tank entered the furnace it had reached a 20 temperature of some 1500 to 1600° F. The valve 17 was closed and a pressure of several inches of water was afterwards maintained by the admission of air. The firing was completed in about three quarters of an hour and the tank was 25 removed from the furnace to cool. Very satisfactory results have been obtained by the use of this method of firing. Defects which frequently occur when air is the atmosphere within the tank are substantially eliminated. 30

I claim:

1. The method of fusing a vitreous enamel lining to the interior of a tank which comprises heating the tank in a furnace with air in the tank in order to form a layer of oxide on the interior of the tank below the coating of enameling material, introducing solid carbon dioxide within the tank to force out the air which it originally contained, maintaining a carbon dioxide atmosphere within the tank until its temperature has 40 risen sufficiently high to fuse the enamel and thereafter admitting air to the tank to maintain within it a pressure in excess of the atmospheric pressure.

2. The method of fusing a vitreous enamel 45 lining to the interior of a tank which comprises heating the tank in a furnace with air in the tank in order to form a layer of oxide on the interior of the tank below the coating of enameling material introducing solid carbon dioxide within 50 the tank to force out the air which it originally contained and maintaining a carbon dioxide atmosphere within the tank until its temperature has risen sufficiently high to fuse the enamel.

3. The method of fusing a vitreous enamel 55 lining to a tank which comprises heating the tank in a furnace with air in the tank, introducing solid carbon dioxide within the tank to force out the air which it originally contained, maintaining a carbon dioxide atmosphere within 60 the tank until its temperature has risen sufficiently high to fuse the enamel, and thereafter admitting air to the tank to maintain within it a pressure in excess of the atmospheric pressure.

4. In the fusing of a vitreous enamel lining to 65 the interior of a tank, the step which comprises replacing air within the tank with another atmosphere by introducing solid particles of the other atmosphere into the tank and thereafter vaporizing them to form a gas.

5. In the fusing of a vitreous enamel lining to 70 the interior of a container, the step which comprises replacing air within the container with another atmosphere while the container is being heated and before it has reached the fusing tem- 75

perature of the enamel, by introducing solid particles of the other atmosphere into the container and thereafter vaporizing them to form a gas.

- 5 6. In the fusing of a vitreous enamel lining to the interior of a container, the step which comprises replacing air within the container with carbon dioxide gas by introducing solid carbon dioxide into the container and thereafter vaporizing it to form carbon dioxide gas.
- 10 7. In the fusing of a vitreous enamel lining to the interior of a container, the steps which comprise heating the container with an oxidizing atmosphere therein to form an oxide film on the inner surface of the container, and thereafter

replacing the atmosphere present in the container with a different atmosphere by introducing solid particles of said different atmosphere into the container and vaporizing them to form gas.

- 5 8. In the fusing of a vitreous enamel lining to the interior of a container, the steps which comprise heating the container with air therein to form an oxide film on the inner surface of the container, and thereafter replacing the air within the container with carbon dioxide gas by introducing solid particles of carbon dioxide into the container and vaporizing them to form carbon dioxide gas.

WESLEY G. MARTIN.